

## UNITED STATES PATENT OFFICE

2,528,782

## LUBRICANT

Orland M. Reiff and Harry J. Andress, Jr., Woodbury, N. J., assignors to Socony-Vacuum Oil Company, Incorporated, a corporation of New York

No Drawing. Application February 8, 1946,  
Serial No. 646,505

9 Claims. (Cl. 252—45)

1

This invention has to do with the art of lubrication and, more particularly, has to do with lubricant compositions.

It is well recognized by those familiar with the art that lubricant compositions, such as viscous mineral oil fractions, tend to deteriorate when used in present day internal combustion engines. In such use, as a result of oxidation of the oil, there is developed appreciable acidity which has a deleterious effect upon metal parts with which the oil is in contact. This is particularly severe in the case of certain types of alloy bearing metals, such as copper-lead, cadmium-nickel, cadmium-silver, and the like. In addition, the lubricating effectiveness of such lubricant compositions may be seriously reduced by virtue of the relatively large change in viscosity at engine operating temperatures.

A great many characterizing or improving agents have been proposed for use in lubricants, such as viscous mineral oil fractions, to counteract the aforesaid undesirable features thereof. For example, many compounds containing sulfur in non-corrosive form have been proposed as oxidation and corrosion inhibitors for such lubricants. One such class is that comprising substituted- and unsubstituted-thiophenes proposed by B. H. Shoemaker and C. M. Loane in Patent No. 2,160,293, issued May 30, 1939. Included among the substituted thiophenes in the foregoing class are alkyl-substituted thiophenes, specifically lauryl, dicyclohexyl, isopropyl, and hexyl thiophenes. As shown in this patent, the aforesaid alkyl-substituted thiophenes are effective for inhibiting corrosion of hard metal alloy bearings. We have now discovered, however, that a certain subclass of alkyl-substituted thiophenes is characterized by an unusually high order of effectiveness in inhibiting lubricants against the deleterious effects of oxidation.

The alkyl-substituted thiophenes contemplated herein are those which contain at least one hydrocarbon wax substituent and may be represented by the following general formula:



wherein  $\text{R}^1$ ,  $\text{R}^2$ ,  $\text{R}^3$ , and  $\text{R}^4$  are either hydrogen or alkyl, aryl, aralkyl or alkaryl groups, and wherein at least one, and as many as all four, of said  $\text{R}$  groups, is a hydrocarbon wax substituent. Typical of such compounds are mono-hydrocarbon wax-thiophene; mono-hydrocarbon wax-di-butylthiophene; di-hydrocarbon wax-thiophene.

The hydrocarbon wax substituent or substituents with which the thiophene compounds of this invention are characterized consist of hydrogen and carbon, as distinguished from ester waxes. The hydrocarbon wax substituent contains at least eighteen carbon atoms in the lowest carbon chain and is derived from a hydrocarbon wax having a melting point varying between about

2

90° F. and about 180° F. Preferred hydrocarbon waxes from which the hydrocarbon wax substituents are derived are those known in the art as the paraffin waxes which contain at least twenty carbon atoms and which have melting points varying between about 90° F. and about 140° F. Outstanding results have been obtained with a particularly preferred paraffin wax, specifically one which contains at least twenty carbon atoms, contains an average of about twenty-four carbon atoms to the molecule, has a melting point of about 126° F. and has a molecular weight of about 350. Other typical hydrocarbon waxes which may be used include the cerese waxes derived from petroleum; these waxes have melting points as high as 180° F.

Any of the methods known in the art for alkylating thiophene may be resorted to for preparing the hydrocarbon wax-substituted thiophenes of this invention. For example, an iodo-thiophene may be condensed with an iodo-substituted wax in the presence of metallic sodium. Wax-substituted thiophenes may also be prepared by reacting thiophenes with a wax olefin 20 in the presence of an activated natural clay or in the presence of a synthetic catalyst containing silica and at least one amphoteric metal oxide, as described in copending application Serial No. 521,866, filed February 10, 1944, now 25 Patent No. 2,448,211, issued August 31, 1948, by P. D. Caesar and A. N. Sachanen. The wax olefin used in the latter method is prepared by dehydrohalogenation of a halogenated hydrocarbon wax, such as by heating the halogenated 30 hydrocarbon with wax at a temperature of about 450° F. in the presence of lime or clay. The wax-substituted thiophenes may be prepared by reacting thiophene with a wax olefin, halide, alcohol or mercaptan in the presence of 35 40 boron trifluoride or certain boron trifluoride complexes, as shown in copending application Serial No. 565,788, filed November 29, 1944, now Patent No. 2,469,823, issued May 10, 1949, by R. C. Hansford and P. D. Caesar. Another suitable 45 method involves reacting an alkyl thiophene, such as butylthiophene, with a wax halide in the presence of a metal halide alkylation catalyst, as described in our copending application Serial No. 580,706, filed March 2, 1945, now Patent 50 No. 2,502,390, issued March 28, 1950, of which the present application is a continuation-in-part.

The preparation and character of the hydrocarbon wax-substituted thiophene of this invention are illustrated by the following typical examples.

## EXAMPLE I

## Paraffin wax-substituted dibutyl thiophene

A mixture consisting of 100 grams of dibutylthiophene, 260 grams chlorinated paraffin wax containing 14 per cent by weight of chlorine (the paraffin wax has a molecular weight of about 350 and a melting point of about 126° F.), and 3 per

cent by weight of anhydrous aluminum chloride, was heated to a temperature of about 350° F. in about one hour while stirring vigorously to avoid foaming induced by the evolution of hydrogen chloride. The mixture was maintained at this temperature for another hour while still stirring to insure complete reaction. Stirring was discontinued when hydrogen chloride was no longer evolved from the mixture. To purify the reaction mixture the latter was cooled to a temperature of 150-200° F., and an amount of water equal to about one quarter the volume of the reaction mixture was added. About 3 percent by weight of zinc dust was then added and the resulting reaction mixture was stirred for about 30 minutes. During this latter treatment, the reaction mixture was decolorized and the aluminum chloride therein was dissolved in the water layer which separated, the water layer was then removed and the remaining reaction mixture was washed with several portions of water. Butanol was used in conjunction with the water to break emulsions which formed. The water-washed reaction mixture was heated to remove the butanol and any residual water. The product thus obtained was predominantly paraffin wax-substituted dibutyl-thiophene and was characterized by the following properties: A. P. I. gravity 24.6; viscosity index 116.9; sulfur content 4.9 per cent by weight; molecular weight 557; pour point (A. S. T. M.) +80° F.

#### EXAMPLE II

##### Paraffin wax-substituted thiophene

A paraffin wax having a melting point of about 126° F., a molecular weight of about 350, and containing at least 20 carbon atoms with an average of 24 carbon atoms, was chlorinated by bubbling chlorine therethrough until the weight of the wax had increased by about 13 per cent. Two hundred grams of the chlorinated paraffin wax so prepared was contacted with 45 grams of lime (CaO) and the resultant mixture was agitated and heated for about 5 hours at about 500° F. Hydrogen chloride was evolved during this treatment and was neutralized, to a large extent, by reaction with the lime thus forming CaCl<sub>2</sub>. The reaction mixture was filtered to remove the CaO-CaCl<sub>2</sub> mixture and to obtain the unsaturated paraffin wax or paraffin wax olefin. The iodine value of the paraffin wax olefin was about 100.

mixture was cooled and filtered to remove the clay catalyst. The filtrate thus obtained was distilled to a maximum temperature of about 400° F. to remove any unreacted thiophene. The reaction product is predominantly mono-paraffin wax thiophene and is characterized by the following: A. P. I. gravity 25.8; viscosity index 137.0; 6.26 per cent sulfur; molecular weight of 456 and a pour point of 80° F.

It will be noted that the pour points of the products obtained in Examples I and II above are relatively high. These materials contain some free paraffin wax and can be dewaxed by the usual methods for dewaxing mineral oil lubricants. The dewaxed materials, those from which substantially all free paraffin wax has been removed, have sufficiently low pour points to be used as synthetic oils. For example, the mono-paraffin wax thiophene prepared in Example II above was dewaxed by diluting the same with 600 per cent by weight of methyl ethyl ketone followed by cooling the resulting mixture to 0° F. and filtering the cooled mixture at 0° F. The filtrate thus obtained was distilled to remove the methyl ethyl ketone and to obtain a product substantially free of paraffin wax. The mono-paraffin wax thiophene thus obtained had a pour point of +20° F.

To demonstrate the unusually high order of effectiveness of the hydrocarbon wax-substituted thiophenes of this invention when used in lubricant compositions, comparative operation tests have been conducted with representative mineral oils alone, with the same oils blended with typical hydrocarbon wax-substituted thiophenes, and with the same oils blended with lauryl (or dodecyl) thiophene disclosed in Patent No. 2,160,293, referred to hereinabove. The test used is the Lauson Engine Test which involves operating a single cylinder Lauson engine for 36 hours at an oil temperature of 290° F. and a jacket temperature of 212° F. The oil used was a solvent-refined oil having a kinematic viscosity of 5.8 centistokes at 210° F. (S. U. V. of 45 seconds at 210° F.), and the oil blends used were blends of said oil and of substituted thiophenes. After 36 hours of test, the acidity, as represented by the neutralization number (N. N.) of the oil blend, and the kinematic viscosity of the oil blend were measured. The results of these tests are tabulated in Table I below.

Table I

| Compound Added                | Alkyl Subst.                              | Conc., Weight Per Cent | K. V. @ 210° F. |               | K. V. Per Cent Change | Ratio, oil: oil Blend | N. N. of Oil | N. N. of oil Blend | Ratio, oil: oil Blend |
|-------------------------------|-------------------------------------------|------------------------|-----------------|---------------|-----------------------|-----------------------|--------------|--------------------|-----------------------|
|                               |                                           |                        | Before Test     | After 36 hrs. |                       |                       |              |                    |                       |
| None                          |                                           |                        | 5.8             | 10.53         | 81.5                  | 1.6                   | 12.9         | 8.8                | 1.5                   |
| Lauryl thiophene              | Lauryl (12 carbon)                        | 5                      | 5.8             | 8.83          | 51.8                  |                       |              |                    |                       |
| None                          |                                           |                        | 5.8             | 9.95          | 71.5                  | 1.7                   | 15.3         | 5.9                | 2.6                   |
| Pentadecyl thiophene          | (pentadecyl 15 carbons)                   | 5                      | 5.8             | 7.53          | 41.7                  |                       |              |                    |                       |
| None                          |                                           |                        | 5.8             | 9.23          | 59.0                  | 1.6                   | 14.3         | 7.1                | 2.0                   |
| Pentadecyl, Dibutyl thiophene | Pentadecyl (15 carb.), 2-butyl (8 carb.)  | 5                      | 5.8             | 7.97          | 37.4                  |                       |              |                    |                       |
| None                          |                                           |                        | 5.8             | 9.95          | 71.5                  | 7.3                   | 15.3         | 2.7                | 5.7                   |
| Monowax Thiophene             | Wax (ave. 24 carb.)                       | 5                      | 5.8             | 6.37          | 9.8                   |                       |              |                    |                       |
| None                          |                                           |                        | 5.8             | 9.23          | 59.0                  | 9.0                   | 14.3         | 1.2                | 12                    |
| Monowax, Dibutyl Thiophene    | Wax (ave. 24 carbons) 2-Butyl (8 carbons) | 5                      | 5.8             | 6.11          | 5.3                   |                       |              |                    |                       |

A mixture of 100 grams of the aforesaid paraffin wax olefin and 30 grams of thiophene was heated in an autoclave at about 400° F. for about 5 hours in the presence of about 10 per cent by weight of a synthetic clay catalyst. The catalyst comprises silica in association with alumina. The reaction

70 It will be apparent from the foregoing tabulation that alkyl-substituted thiophenes, such as lauryl and pentadecyl, are somewhat effective in retarding acid formation and viscosity change; however, this effectiveness is several times less than the effectiveness of the wax-substituted

thiophenes, such as monowax and monowax dibutyl thiophene. For example, oil blends containing lauryl, pentadecyl and pentadecyl dibutyl thiophenes are only about 1.6-1.7 times better than the uninhibited oil (i. e., free from a substituted thiophene) on the basis of retarding viscosity change; whereas on the same basis, monowax and monowax dibutyl thiophenes, respectively, are 7.3 and 9.3 times better than the uninhibited oil. The superiority of the wax compounds is similar when based upon retardation of acid formation: 1.5-2.6 for the non-wax compounds and 5.7-12 for the wax compounds.

The cerese wax-substituted thiophenes have been found to be effective pour point depressants. For example, a cerese wax-substituted dibutyl thiophene, when used in 1/2% and 1% concentrations in a mineral oil of +20° F. pour point, depressed the pour point to -5° F. and -15° F. respectively.

The wax-substituted thiophenes are miscible in all proportions with mineral oils and as such, may be used therein in all proportions. They may be used therein as corrosion and oxidation inhibitors, for example, in concentrations of the order of from about one per cent to fifty per cent, with satisfactory results generally obtained with about 5-20 per cent. They may also be used in other lubricants such as fatty oils, including corn oil, soy-bean oil, lard oil, and the like. Further, they may be blended with volatalized oils, synthetic oils or greases. Moreover, they may be used in oils in conjunction with other additive materials such as pour point depressants, viscosity index agents, oiliness agents, and the like.

It is to be understood that the present invention is not to be construed as limited to the foregoing illustrative examples, but it is to be construed broadly in the light of the language of the appended claims.

We claim:

1. A mineral lubricating oil containing a minor proportion, sufficient to stabilize said oil fraction against the deleterious effects of oxidation, of an anti-oxidant material the essential anti-oxidizing ingredient of which is a hydrocarbon wax-substituted thiophene represented by the general formula:



wherein R<sup>1</sup>, R<sup>2</sup>, R<sup>3</sup> and R<sup>4</sup> are selected from the group consisting of hydrogen and alkyl and at least one of said R groups is a hydrocarbon wax group.

2. A mineral lubricating oil containing a minor proportion, sufficient to stabilize said oil fraction against the deleterious effects of oxidation, of an anti-oxidant material the essential anti-oxidizing ingredient of which is a hydrocarbon wax-substituted thiophene represented by the general formula:



wherein R<sup>1</sup>, R<sup>2</sup>, R<sup>3</sup> and R<sup>4</sup> are selected from the group consisting of hydrogen and alkyl and at least one of said R groups is a hydrocarbon wax group containing at least about 20 carbon atoms.

3. A mineral lubricating oil containing a minor proportion, sufficient to stabilize said oil fraction against the deleterious effects of oxidation, of an anti-oxidant material the essential anti-oxidizing ingredients of which is a hydrocarbon

wax-substituted thiophene represented by the general formula:



wherein R<sup>1</sup>, R<sup>2</sup>, R<sup>3</sup> and R<sup>4</sup> are selected from the group consisting of hydrogen and alkyl and at least one of said R groups is a hydrocarbon wax group containing at least about 20 carbons and having an average of about 24 carbon atoms.

4. A mineral lubricating oil containing a minor proportion, from about one per cent to about 20 per cent, of a hydrocarbon wax-substituted thiophene represented by the general formula:



wherein R<sup>1</sup>, R<sup>2</sup>, R<sup>3</sup> and R<sup>4</sup> are selected from the group consisting of hydrogen and alkyl and at least one of said R groups is a hydrocarbon wax group.

5. A mineral lubricating oil containing a minor proportion, sufficient to stabilize said oil fraction against the deleterious effects of oxidation, of an anti-oxidant material the essential anti-oxidizing ingredient of which is a poly-hydrocarbon wax-substituted thiophene.

6. A mineral lubricating oil containing a minor proportion, sufficient to stabilize said oil fraction against the deleterious effects of oxidation, of an anti-oxidant material the essential anti-oxidizing ingredient of which is a mono-hydrocarbon wax-substituted thiophene.

7. A mineral lubricating oil containing a minor proportion, sufficient to stabilize said oil fraction against the deleterious effects of oxidation, of an anti-oxidant material the essential anti-oxidizing ingredient of which is a mono-hydrocarbon wax substituent containing at least about 20 carbon atoms and having an average of about 24 carbon atoms.

8. A mineral lubricating oil containing a minor proportion, sufficient to stabilize said oil fraction against the deleterious effects of oxidation, of an anti-oxidant material the essential anti-oxidizing ingredient of which is a dibutyl thiophene containing at least one hydrocarbon wax substituent attached to a carbon atom of the thiophene nucleus.

9. A mineral lubricating oil containing a minor proportion, sufficient to stabilize said oil fraction against the deleterious effects of oxidation, of an anti-oxidant material the essential anti-oxidizing ingredient of which is a dibutyl thiophene containing at least one hydrocarbon wax substituent attached to a carbon atom of the thiophene nucleus, said hydrocarbon wax substituent containing at least about 20 carbon atoms and having an average of about 24 carbon atoms.

ORLAND M. REIFF.  
HARRY J. ANDRESS, JR.

#### REFERENCES CITED

The following references are of record in the file of this patent:

#### UNITED STATES PATENTS

| Number    | Name        | Date          |
|-----------|-------------|---------------|
| 2,141,611 | Malishev    | Dec. 27, 1938 |
| 2,160,293 | Shoemaker   | May 30, 1939  |
| 2,258,806 | Pier et al. | Oct. 14, 1941 |
| 2,429,575 | Appleby     | Oct. 21, 1947 |